

July 30, 1963

R. B. HURLEY ET AL

3,099,517

PROCESS OF TREATING WET-SPUN ACRYLONITRILE POLYMER FIBERS

Filed Dec. 16, 1960

2 Sheets-Sheet 1



Fig. 1



Fig. 2



Fig. 3



Fig. 4



Fig. 5

INVENTORS.

Rupert B. Hurley  
Paul C. Colodny

BY Jerome R. Hurley  
ATTORNEY

July 30, 1963

R. B. HURLEY ET AL

3,099,517

PROCESS OF TREATING WET-SPUN ACRYLONITRILE POLYMER FIBERS

Filed Dec. 16, 1960

2 Sheets-Sheet 2



Fig. 6



Fig. 7



Fig. 8



Fig. 9



Fig. 10

INVENTORS.  
Rupert B. Hurley  
Paul C. Colodny

BY  
Rupert Hurley  
ATTORNEY

## 1

3,099,517

## PROCESS OF TREATING WET-SPUN ACRYLO-NITRILE POLYMER FIBERS

Rupert B. Hurley, Williamsburg, Va., and Paul C. Colodny, Carmichael, Calif., assignors to The Dow Chemical Company, Midland, Mich., a corporation of Delaware

Filed Dec. 16, 1960, Ser. No. 76,219  
12 Claims. (Cl. 18—48)

The present invention resides in the field of synthetic textile fibers and contributes to the art of their manufacture. More precisely, it relates to a useful and advantageous process for stretching or orienting wet-spun acrylonitrile polymer fibers while they are in an aquagel state that are prepared by being coagulated from suitable spinning solutions or equivalent compositions (such as spinable dispersions) in aqueous coagulating spin baths and subsequently washed with water to remove residual spinning solution solvent from the freshly wet spun fiber.

The invention has particular reference to the manufacture of acrylonitrile polymer fibers which are fabricated from fiber-forming acrylonitrile polymers that contain in the polymer molecule at least about 80 weight percent of polymerized acrylonitrile, especially polyacrylonitrile, which are wet spun in and with systems that are adapted to utilize aqueous coagulating liquids for the spinning operation, such as systems wherein ethylene glycol, dimethyl formamide, dimethyl sulfoxide, butyrolactone and the like or the various aqueous saline polyacrylonitrile-dissolving solvents are employed as spinning solution solvents for the polymer and are also present in non-polymer-dissolving quantities in the aqueous coagulating liquid used in the spin bath.

The utile, known aqueous saline solvents for the various fiber-forming acrylonitrile polymers and polyacrylonitrile include zinc chloride, the various thiocyanates such as calcium, lithium bromide, salt mixtures of the so-called "lyotropic" series, and others recognized by the art, as has been disclosed, among other places, in United States Letters Patents Nos. 2,140,921; 2,425,192; 2,648,592; 2,648,593; 2,648,646; 2,648,648; 2,648,649; and 2,949,435. Advantageously, aqueous zinc chloride solutions are used for the purpose.

It is common knowledge to the man-made fiber art that most of the synthetic fibers must be stretched or oriented sometime during their manufacture. Depending on the crystallinity and/or molecular configuration of the fiber, the amount of stretching and stretching conditions may differ widely. In some cases very little stretch is necessary, in others, the fibers may be stretched as much as 1300–2000 percent. The stretching may be done cold or hot, in air, water or some other gaseous or liquid medium. In all cases the intent is to align to some extent the crystallites or polymer molecules parallel to the fiber axis. This alignment is necessary in order to take advantage of the inherent tensile properties in the fibers.

Wet spinning of fibers generally involves spinning a solution of a polymer dissolved in a solvent for the polymer into a non-polymer-dissolving liquid causing a polymeric filament to coagulate. The polymer solvent is thus washed or leached out of the coagulated polymer and most often replaced with an inert liquid, frequently water. The filament so formed is usually in a gel state, that is, it is highly swollen and may contain as much as 4–6 times as much non-polymer-dissolving or inert liquid, e.g., water, as polymer. The gel filament is usually washed, stretched, and, ultimately, dried to destroy the gel structure.

It is also well established in the art that the stretching or orienting of acrylonitrile polymer wet-spun fibers is

## 2

usually done at temperatures in the range of 70°–110° C., and preferably at 90–100° C. in the presence of moisture. Ordinarily, high stretch ratios are only possible at the higher temperatures if undue filament breaking is to be avoided; and, stretch ratios of about 10:1 and higher are normally necessary to produce fibers with a satisfactory combination of physical properties. The total stretch given the fiber has been imparted in one step or in several sequential increments.

10 However, in the prior art, no particular attention has been paid to the sequence of stretching as associated with temperature, the principal interest lying solely in the desired ultimate stretch imparted to the fibers. Thus, any physical-property improvements in the fibers resulting 15 from the stretch were dependent on the total stretch ratio applied to the fibers. It remained, then, that avenues pursued to improving or altering the fiber physical properties that could not be obtained through stretch ratios were those such as changing the polymer composition, 20 e.g. forming copolymers, and certain other treatments performed on the fibers after they had been substantially oriented, or after they had been oriented and dried.

It is the prime interest and concern of this invention to 25 provide a process whereby in a continuous and consistently uniform manner wet-spun acrylonitrile polymer fibers can be made to have greatly improved physical properties without having to require the use of extreme alterations in normal wet-spinning techniques. In particular, 30 it is an object of this invention to provide wet-spun acrylonitrile polymer fibers with increased physical properties by utilizing an especially advantageous process for stretching the substantially unstretched fibers while they are in the gel state.

35 This invention takes advantage of the criticalities of the temperature-stretching sequence used during the stretching or orienting of wet-spun acrylonitrile polymer gel fibers. In accordance with this invention, highly improved physical properties of the fibers can be obtained 40 by; prior to imparting any substantial stretch to the gel fibers, i.e., less than about 1.5:1, they are contacted with an aqueous medium at a temperature of from about 50° to about 80° C. (for at least about 2 seconds); setting the gel structure; and subsequently stretching said gel fibers 45 while they are exposed to a heated medium maintained at from about 80° to about 110° C.

The treatment according to the invention, which in part might be best referred to as a gel-structurizing treatment, 50 is thought to impart a particular morphological structure to the gel which in turn is thought to be responsible for the new improved and distinct properties of the resulting fiber. The change in structure is observable when a typical stress-strain curve is run on the gel treated as prescribed by the invention. It is essential for satisfactory practice of the invention that this particular and beneficially imparted gel structure be "set" in the gel filament 55 before any stretch is given to the filament at temperatures above about 80° C.

60 The setting of the structure can be accomplished by one of two methods: (1) The structure can be set by stretching the gel filament while the filament is being subjected to the gel-structurizing treatment, that is, while being contacted with an aqueous medium at 50°–80° C. 65 Any permanently elongating stretch is sufficient to set the gel. A stretch ratio of 1:1.1 may be employed, but ratios of from about 2:1 to about 8:1 are more advantageous. (2) The filament may be removed from the gel-structurizing medium held at 50°–80° C., more advantageously at 55°–75° C., and cooled to some temperature below that at which the gel-structurizing medium was maintained. The aqueous gel-structurizing medium is prefer-

ably essentially water but may contain other water-miscible materials inert to the gel filament, or other water-miscible or dispersible beneficial adjuvants desirous of being impregnated into the gel.

After either method, the fiber is then stretched in a subsequent heated medium at 80° to 110° C., preferably at 90° to 110° C., and advantageously at 95° to 100° C. A single subsequent stretch at 80°-110° C. or a sequential series of stretches at 80-110° C. may be employed. Either a liquid aqueous bath or a gaseous or vapor atmosphere such as saturated steam may be employed as the stretching medium.

In practicing the present invention, the gel structure imparted to the gel filaments or the change in the gel structure is irreversibly introduced as long as the structure is set by one of the methods hereinbefore set forth. For example, if a gel filament is treated at 70° C. and then cooled to 60° C. or lower and stretched, the gel structure will have the characteristics of the 70° C. temperature treatment. The filament would have the same characteristics if stretched while being treated at 70° C. On the other hand, if a fiber were treated at 70° C. and then heated to 80° C. and stretched, the effects of the 70° C. treatment would be erased and the 80° C. treatment characteristics would prevail. In all cases, the highest temperature at which the gel structure is introduced, provided the structure is "set" at that or a lower temperature, will dominate the characteristics of the gel filament, and hence the physical properties of the resulting finally converted textile fiber. If a treating or gel-structurizing temperature is employed below about 50° C., no physical-property-improving characteristics are introduced into the gel. Similarly, but with different end results, above about 80° C., although a structure is introduced which has an effect on the physical properties, the improvements are not evidenced that are brought about by treating in the range of 50-80° C. It should be made clear that the benefits of this invention are not evidenced by a transient pass of the gel filaments through an aqueous medium at 50°-80° C. to a higher temperature without a setting step. In other words, the treatment must be interrupted by either cooling to some lower temperature or stretching before exposing to a higher temperature.

As previously indicated, the characteristic change introduced into the gel structure by the 50-80° C. temperature treatment can be identified through observing a stress-strain curve obtained from a simultaneously recorded tensile test on the unstretched gel filament. (Frequently, a slight stretch of about 1.4:1 at 20-25° C. may be given the gel filaments after they are coagulated to give them enough strength for subsequent processing, but for all practical purposes, the filaments are referred to as unstretched.)

FIGURE 1 represents a typical stress-strain curve obtained from an unstretched wet-spun polyacrylonitrile gel filament that was treated in a water bath at 20°-25° C.

FIGURE 2 represents a typical stress-strain curve obtained from an unstretched gel filament from the same sample as the filament used for FIGURE 1 but which had been treated in a water bath within the temperature range in accordance with the invention.

From a comparison of the typical curves of FIGURES 1 and 2, it is seen that an unusual "peaking" of the initial slope on the curve and then a falling back to the normal stress-strain curve itinerary is characteristic to gel filaments produced according to the invention. This "peaking" and return to the more usual post slope is absent in the curve of FIGURE 1. Fibers made from gel filaments exhibiting this "peaking" type of stress-strain curve have highly improved physical properties as compared to fibers made from gel filaments with a stress-strain curve shaped like that in FIGURE 1.

The fibers produced according to the invention have highly improved tenacity, yield point, modulus, and transverse properties. One measure of improved transverse

properties are the improved wet fibrillation properties of the fiber. In addition, it is frequently desirable to impregnate the gel (or aquagel) filaments with a dye additive, and, the instant process reduces the required amount of dye additive to obtain the same dyeability when contrasted to the stretching process common to the usual practice. Similarly, impregnation with other beneficial adjuvants is improved.

General wet spinning techniques involve, in sequence; 10 extruding the polymer dissolved in a suitable aqueous solvent or water-miscible solvent, coagulating to a polymeric gel filament, washing the filament essentially completely free of residual solvent, imparting the desirable stretch or orientation to the filament, possibly followed by 15 other miscellaneous treatments, and finally irreversibly drying the gel structure to a characteristic textile fiber.

In the practice of this invention, the gel-structurizing treatment is preferably performed succeeding the washing step and necessarily preceding or partially simultaneously 20 with the stretching or orienting step.

After their extrusion, coagulation, washing, gel-structurization and gel setting, the freshly wet spun filaments may be subsequently handled and treated in any desired or necessary manner for purposes of converting them to 25 a finished fiber product. Thus, they may be stretched or otherwise treated for purposes of heat treating or relaxing the fibers in any desired way or they may be subjected to additional treatments of any appropriate nature, including application of finishes, lubricants and the like or imposition of crimp prior to being dried and finally collected as completely manufactured products.

As has been indicated, when acrylonitrile polymer, particularly polyacrylonitrile, fibers are being manufactured, zinc chloride may most advantageously be utilized as the 30 sole, or at least the principal, saline solute in the spinning solvent employed for the polymer. In such instances, the aqueous solution of zinc chloride in the spinning solution may advantageously be in a concentration of from 55 to 65, preferably about 60 percent by weight, based on the 35 weight of the aqueous solution. When such aqueous zinc chloride solvent spinning solutions are employed, it is desirable to maintain the concentration of zinc chloride in the portion of the liquid in the spinning zone at a non-polymer-dissolving coagulating concentration of at least 40 25 percent by weight; advantageously from about 30 to 50 percent by weight, and preferably between about 40 and 45 percent by weight. In such aqueous zinc chloride systems for acrylonitrile polymers, wherein the freshly wet spun polymer is generally obtained in an aquagel form, it 45 is generally desirable for the spinning solution that is extruded to contain between about 4 and 20 percent by weight of dissolved polymer; more advantageously from about 6 to 15 percent by weight of dissolved polymer; and preferably, particularly when polyacrylonitrile fibers are 50 being manufactured, from about 8.5 to 11.5 percent by weight of fiber-forming polymeric solids in the spinning solution.

Aqueous zinc chloride spinning solutions of fiber-forming acrylonitrile polymers are beneficially extruded at a 55 spinning temperature of from 0 to 50° C.; preferably from about 10 to 30° C., into an aqueous zinc chloride coagulating liquid that is maintained at a coagulating temperature of from 0 to 30° C.; preferably from about 10 to 20° C. Thoroughly washed acrylonitrile polymer aquagel fibers, 60 incidentally, are usually found to contain not more than 5½ parts by weight of water (including residual extrinsic or exterior water associated therewith) for each part by weight of dry polymer therein. More frequently, washed acrylonitrile polymer aquagel fibers are found to contain 65 from about 2 and usually from about 3 to 4 parts by weight of water for each part by weight of polymer.

Homopolymeric acrylonitrile gel filaments or polymeric gel filaments formed from copolymerizing acrylonitrile with one or more other ethylenically unsaturated monomers copolymerizable with acrylonitrile such that the 70

copolymeric product contains at least about 80 percent by weight of acrylonitrile polymerized in the polymer molecule may be beneficially and advantageously treated according to this invention. Examples of other monomeric materials which may be employed advantageously with acrylonitrile in the practice of the present invention include allyl alcohol, vinyl acetate, acrylamide, methacrylamide, methyl acrylate, 2-vinyl pyridine, dimethylaminomethylacrylate, methacrylonitrile, acrylic acid, itaconic acid, vinyl acetic acid, ethyl acrylate, fumaronitrile, 2-vinyl 5-ethyl pyridine, ethylene sulfonic acid and its alkali metal salts, allyl sulfonic acid and its alkali metal salts, vinyl lactams such as vinyl caprolactam and vinyl piperidone, vinyl benzene sulfonic acid and its salts, vinylbenzene-trimethyl ammonium chloride, vinylmethyl ether, N-acryloyltaurine and its salts, 2-amino-ethyl-methacrylate hydrochloride, 2-sulfoethylacrylate, X-sulfopropylacrylate, maleic anhydride and the like, including mixtures thereof.

In addition, the properties of certain other of the modified acrylonitrile polymer fibers may be beneficially enhanced by practice of the present invention, especially those that are comprised of the essential acrylonitrile polymer base, particularly polyacrylonitrile, in which there has been intimately and permanently or substantially permanently incorporated minor proportions of from 1 or 50 up to about 20 or so percent by weight, based on the weight of the polymeric composition of any of the beneficial additaments or constituents adapted to serve the desired purpose and provide the beneficial result. These referred-to polymeric compositions are frequently called "acrylic alloys." Generally, such beneficial additaments are employed primarily as dye-assisting adjuvants or components. Advantageously, they may be the polymerized products of such azotic monomers, or mixtures thereof, as the several N-vinyl lactams including such broadly related products as the N-vinyl-2-morpholinones; the N-vinyl-2-oxazolidinones; and certain of the N-vinyl-N-methyl-alkyl-sulfonamides.

Thus, the acrylic alloy may be comprised of the acrylonitrile polymer base that is prepared by graft or block copolymerization of acrylonitrile or an acrylonitrile containing monomer mixture upon a minor proportion of an already formed polymer derived from any of the indicated varieties of azotic monomers or their mixtures. Or, as mentioned, it may consist of a graft copolymer product of any of the indicated varieties of azotic monomers on an already formed and preferably already fabricated acrylonitrile polymer base.

Advantageously, and frequently with consummate suitability, the acrylic alloy fiber may be comprised of the acrylonitrile polymer base in which there is permanently incorporated by physical blending in minor proportion of any of the polymer products from the specified azotic monomers or mixtures thereof, primarily as dye-assisting adjuvants. The physical blending can be carried out prior to spinning of the fiber-forming solution, or as in the case of wet spinning, it can profitably be incorporated in the aquagel filament prior to irreversibly drying the aquagel.

As indicated, the adjuvant or beneficial constituent in the acrylic alloy fiber may be homopolymeric in nature or it may be a straight copolymer of any of the azotic monomers specified with other mono- and polyfunctional monomers. Adjuvants of this variety are ordinarily physically blended with the essential acrylonitrile polymer base in order to secure the desired intimate incorporation of the beneficial constituent and the resulting alloying effect in the fiber. Likewise, there may be similarly utilized for physical blending purposes adjuvants or additaments that are graft copolymeric in nature and which consist of various monomers that are graft copolymerized on substrates consisting of polymers of any of the indicated azotic monomers, such as poly-N-vinylactam substrates; poly-N-vinyl-2-oxazolidinone substrates and poly-N-vinyl-N-methyl-alkylsulfonamide substrates. Similarly, just

as suitably, graft copolymeric additaments may be provided and employed when they consist of any of the specified or closely related azotic monomers (such as N-vinyl-lactam monomers, N-vinyl-2-oxazolidinone monomers and N-vinyl-N-methyl alkylsulfonamide monomers graft copolymerized on other functional polymer substrates.

It is usually beneficial for the polymer products of the azotic functional monomers to be present as the beneficial component in acrylic alloy fibers in an amount that is in the neighborhood or range of from about 5 to 15 percent by weight, based on the weight of the acrylic alloy composition. It is frequently quite desirable to employ a homopolymeric N-vinylactam polymer, such as poly-N-vinyl-pyrrolidone (which may also be identified as poly-N-vinyl-2-pyrrolidone or, with varied terminology, poly-N-vinyl-2-pyrrolidinone), poly-N-vinyl caprolactam, or somewhat related thereto, a poly-N-vinyl-3-morpholine; or a homopolymeric N-vinyl-2-oxazolidinone or poly-N-vinyl-5-methyl-2-oxazolidinone; or a homopolymeric N-vinyl-methylalkylsulfonamide polymer such as homopolymeric N-vinyl-N-methyl-methylsulfonamide; as the polymeric adjuvant that is blended with the essential acrylonitrile polymer base in the acrylic alloy composition. When physically blended acrylic alloy products are prepared that utilize, as the beneficial additament or constituent, copolymeric or graft copolymeric products of the indicated azotic monomers, it is usually beneficial for the polymeric adjuvants that are employed to be those which are comprised of at least about 50 percent or even as much as 80 or more percent by weight of the products of the indicated constituents derived from the azotic monomers.

Further features and advantages of the invention will be evident from the following examples, which are presented with no intent of restricting or limiting the invention thereto. Unless otherwise indicated, all parts and percentages are by weight.

#### EXAMPLE 1

In order to exemplify the applicability of the invention over a broad range of conditions, fibers were wet spun using widely differing conditions and then conditioned, or in contrast not conditioned, in accordance with the invention.

A spinning solution was prepared comprised of polyacrylonitrile with an average molecular weight between about 30 and 35 thousand dissolved in an aqueous 60 percent by weight solution of zinc chloride. The total polymer solids in the spinning solution were about 10 percent by weight, based on the weight of the solution. Two sets of coagulating bath conditions were used for spinning the filaments:

An aqueous 47 percent by weight zinc chloride bath maintained at a temperature of 24° C. Filaments spun into this bath were designated sample "A."

An aqueous 43.4 percent by weight zinc chloride bath maintained at a temperature of 11° C. Filaments spun into this bath were designated sample "B." The spinning solution was extruded into each of the coagulating baths,

the coagulated gel filaments were washed essentially free of residual salt, given a stretch of about 1.45:1 at room temperature and collected. The gel filaments of sample "B" were more dense than those of sample "A."

Individual gel filaments from each of samples "A" and "B" were selected at random and subjected to a tensile test at room temperature. The gel fibers were kept under ethylene glycol during the testing to prevent the gel from drying. Stress-strain curves were automatically recorded during the tensile test which is the widely known and accepted procedure for determining the physical properties of fibers and filaments. Five filaments were run from each sample. In FIGURE 3 is seen a typical stress-strain curve representing the curves obtained from the gel filaments of sample "A." Likewise, FIGURE 4 shows a typical stress-strain curve obtained from the gel filaments of sample "B."

Other filaments were selected at random from sample "B" and subjected to a tensile test from which stress-strain curves were simultaneously obtained as described above, except, prior to being tested, they were each placed in a water bath each at a different temperature for a constant period of time, cooled back to room temperature, and then tested. Thus, the gel filaments were given a gel-structurizing treatment, some within the temperature range of the invention, and some without the range. FIGURES 5 through 10 show representative curves typical of those obtained from the treated and tested filaments. Again, five filaments were tested for each sample. The results are summarized in Table I.

Table I

| Figure | Sample            | Temperature of Gel-Structurizing Water Bath (° C.) | Tenacity (grams) | Extension (percent) | Yield (grams) | Modulus (grams) |
|--------|-------------------|----------------------------------------------------|------------------|---------------------|---------------|-----------------|
| 5      | "B <sub>1</sub> " | 50                                                 | 7.0              | 410                 | 4.2           | 2.0             |
| 6      | "B <sub>2</sub> " | 52                                                 | 7.6              | 400                 | 5.8           | 1.0             |
| 7      | "B <sub>3</sub> " | 62                                                 | 7.6              | 400                 | 6.4           | 0.8             |
| 8      | "B <sub>4</sub> " | 72                                                 | 8.4              | 170                 | 11.0          | 2.0             |
| 9      | "B <sub>5</sub> " | 82                                                 | 11.6             | 18                  | 13.2          | 2.0             |
| 10     | "B <sub>6</sub> " | 100                                                | 12.0             | 10                  | 12.0          | 3.1             |
| 3      | "A"               | ca. 20                                             | 3.8              | 440                 | 2.2           | 0.25            |
| 4      | "B"               | ca. 20                                             | 6.7              | 420                 | 4.3           | 2.5             |

The typical curves in FIGURES 3 and 4 (samples "A" and "B"), which can be considered as obtained from gel filaments treated at about 20° C. prior to testing, and the typical curve in FIGURE 5 (sample "B<sub>1</sub>"), obtained from gel filaments treated at 50° C., do not exhibit any "peaking" of the initial slope as exhibited in the curves of FIGURES 6 through 8 (samples "B<sub>2</sub>", "B<sub>3</sub>" and "B<sub>4</sub>"), obtained from gel filaments treated at 52°-72° C. The typical curves of FIGURES 9 and 10 (samples "B<sub>5</sub>" and "B<sub>6</sub>"), obtained from gel filaments treated at 82° C. and 100° C., exhibit a "peaking" of the initial slope but do not exhibit a post slope such as those prominent in FIGURES 6 through 8.

The summation of physical property data in Table I is evidential of the fact that the most advantageous and beneficial combination of physical properties and of improvements in physical properties lie in the gel filaments that have been treated in accordance with the invention, and as a consequential corollary, those that are characterized in an abnormal "peaking" in their stress-strain curves and subsequent return to a normal post slope.

Similar excellent results were obtained when gel filaments from sample "A" were treated in water baths as was done with gel filaments from sample "B". Significant improvements were obtained in physical properties from the filaments treated in conformance with the invention, which filaments also exhibited the "peaking" effect in their stress-strain curves.

## EXAMPLE 2

Gel filaments from sample "B" of Example 1 were treated for 1 minute and 10 minutes in a water bath at 65° C. and then cooled back to room temperature prior to being subjected to a tensile test. The results are shown in Table II.

Table II

| Time of Treatment (Minutes) | Tenacity (grams) | Extension (percent) | Yield (grams) | Modulus (grams) |
|-----------------------------|------------------|---------------------|---------------|-----------------|
| 1                           | 7.2              | 290                 | 5.8           | 3.0             |
| 10                          | 7.8              | 350                 | 7.4           | 2.0             |

Although the results of Table II show slightly improved results for the longer treating time, for all practical purposes, the time is not particularly critical, since significant improvements are obtained when the treatment is imparted for only a few seconds, i.e., 5-10 seconds.

8  
EXAMPLE 3

Polyacrylonitrile fibers were spun from a spinning solution as described in Example 1. They were coagulated in an aqueous 44.5 percent by weight ZnCl<sub>2</sub> solution at 12° C., washed free of residual salt, given a 1.45:1 stretch at room temperature, and then passed through two aqueous baths at 95-100° C. The filaments were stretched 3.4:1 in the first of the two baths and 2.4:1 in the second bath. The total stretch was about 11.88:1. The gel fibers were then irreversibly dried at 140° C. for about 7 minutes to characteristically hydrophobic textile fibers. The final fibers, designated sample "C," were then tested for physical properties including the tendency of the fibers to split off or peel back fibrils from the fiber surface, commonly referred to as wet fibrillation.

Two other fiber samples, samples "D" and "E," were prepared in the same way as sample "C," except the conditions of the hot-wet stretching were changed to conform with the treatment of the invention. Sample "D" was passed through an aqueous bath at 69° C. and stretched 5.39:1 in the bath, and then through two aqueous baths at 95-100° C., being stretched 1.35:1 in the first bath and 1.19:1 in the second bath. The total stretch of sample "D" was about 12.5:1.

Sample "E" was stretched 5.16:1 in a 67° C. aqueous bath and 1.32 in 95-100° C. aqueous bath. The total stretch of sample "E" was about 10:1. The physical properties of samples "D" and "E" were determined as well as wet fibrillation tendencies.

In further contrast, fibers were produced according to the procedure of sample "D" except that a hot stretch of 5.3:1 was given in an aqueous 67° C. bath and no 95-100° C. stretch followed. This sample was designated sample "F." The total stretch of sample "F" was about 8:1.

The results of these four samples are given in Table III.

Table III

| Sample | Tenacity, grams/denier | Extension (percent) | Yield, grams/denier | Modulus |
|--------|------------------------|---------------------|---------------------|---------|
| "C"    | 4.2                    | 30                  | 1.10                | 45      |
| "D"    | 5.8                    | 31                  | 1.33                | 60      |
| "E"    | 5.0                    | 34                  | 1.28                | 64      |
| "F"    | 2.9                    | 34                  | 1.13                | 42      |

As mentioned previously, the resistance to wet fibrillation of samples "C", "D," and "E" were measured. This was determined through a standardized test which involves the use of a Waring Blender for wet fibrillating the fibers. More precisely, samples of fiber are cut to about 1/2 inch staple length and weighed into 200 mg. lots for the standardized test procedure.

After the samples are cut and weighed the flow time for passage of one liter of water through a pad of the material is determined. The pad of fibers is formed by pouring water through a 3/4" diameter by 3" cylinder with a screened bottom and a weighted screen top. Three passes of 300 ml. of water through the device serves to make a uniform pad of the fiber over the screen.

Next, the cylinder containing the sample is placed in the bottom of the container which holds the water for the flow test and the flow time for the one liter of water to pass through the sample is determined with a stop watch.

When the initial flow time has been determined, the sample is now ready for the Waring Blender. The sample is washed from the cylinder and sufficient water added to make up 100 ml. Standard testing calls for 10 minutes' operation, with 100 ml. water, and 75 watts power input to the blender. This treatment is then followed by another flow time measurement and the percent change in flow time recorded as the test result. Thus, the test is based

on the principle that the more fibrillated the fibers the more dense will be the pad of fibers and hence the more resistance offered to the flow of water therethrough.

The resistance to wet fibrillation of samples "D" and "E" were about two times and about four times, respectively, improved over sample "C."

As further exemplification of the benefits of the invention; a sample was prepared the same as sample "C" and poly-N-vinyl-2-pyrrolidone (PVP) was impregnated in the aquagel filaments in the hot stretch baths; approximately 7 percent PVP, based on the weight of the dry fiber, (OWF) was required to obtain a reflectance value of 21 when the fibers were dyed with 2 percent (OWF) Calcodur Pink 2BL (Colour Index Direct Red 75). In contrast, when PVP was put into the hot stretch baths and the filaments treated according to the procedure of sample "D," only 3.48 percent PVP (OWF) was required to obtain a reflectance value of 21.

The dyeing with Calcodur Pink 2BL was performed at the 2 percent level according to conventional procedure in which the fiber sample was maintained for about one hour at the boil in the dye bath which contained the dye-stuff in an amount equal to about 2 percent of the weight of the fiber. The dye bath also contained sodium sulfate in an amount equal to about 15 percent of the weight of the fiber and had a bath-to-fiber weight ratio of about 30:1, respectively. After being dyed, the fiber was rinsed thoroughly with water and dried for about 20 minutes at 80° C. The dye-receptivity of the Calcodur Pink 2BL-dyed fiber was then evaluated spectrophotometrically by measuring the amount of monochromatic light having a wave length of about 520 millimicrons from a standard source that was reflected from the dyed sample. A numerical value on an arbitrarily designated scale from 0 to 100 was thereby obtained. This value represented the relative comparison of the amount of light that was reflected from a standard white tile reflector that had a reflectance value of 316 by extrapolation from the 0-100 scale. Lower reflectance values are an indication of better dye-receptivity in the fiber. For example, a reflectance value of about 20 or 25 to 50 or so for acrylonitrile polymer fibers dyed with 2 percent Calcodur Pink 2BL is generally considered by those skilled in the art to be representative of a degree of dye-receptivity that readily meets or exceeds the most rigorous practical requirements and is ordinarily assured of receiving general commercial acceptance and approval.

Commensurate excellent results to the foregoing are obtained when other acrylonitrile polymer gel fibers, including acrylonitrile polymers of the copolymeric variety or those of the acrylic alloy variety, are treated in accordance with this invention which is encompassed in the hereto appended claims.

What is claimed is:

1. In the method of wet spinning acrylonitrile polymer fibers which are fabricated from fiber-forming acryloni-

trile polymers that contain in the polymer molecule at least about 80 weight percent polymerized acrylonitrile, any balance being another copolymerized ethylenically unsaturated monomer that is polymerizable with acrylonitrile, the improvement which comprises; contacting substantially unstretched acrylonitrile polymer gel fibers with an aqueous medium at from about 50° C. to about 80° C.; setting the gel structure imparted to said acrylonitrile polymer gel fibers by means of cooling said gel fibers to a temperature below the temperature at which said aqueous contacting medium is maintained; and subsequently stretching said gel fibers while they are exposed to a heated medium from about 80° C. to about 110° C.

2. The method of claim 1, wherein said aqueous medium for contacting said acrylonitrile polymer gel fibers is maintained at between about 55° C. and 75° C.

3. The method of claim 1, wherein said medium for contacting said acrylonitrile polymer gel fibers is essentially water.

4. The method of claim 1, wherein said heated medium for said subsequent stretch is maintained at between about 95° C. and 100° C.

5. The method of claim 1, wherein said heated medium is an aqueous medium.

6. The method of claim 1, wherein said heated medium is saturated steam.

7. The method of claim 1, wherein said heated medium is water containing a minor proportion of a vinyl lactam polymer.

8. The method of claim 1, wherein said acrylonitrile polymer is polyacrylonitrile.

9. The method of claim 1, and including the step of irreversibly drying said gel fibers.

10. The method of claim 1, wherein said acrylonitrile gel fibers are spun from an aqueous saline solvent for said acrylonitrile polymer.

11. The method of claim 10, wherein said aqueous saline solvent is an aqueous solution of which the principal saline constituent is zinc chloride.

12. The method of claim 10, and including coagulating said acrylonitrile polymer gel fibers in a bath comprising the same saline constituents that are present in said aqueous saline solvent.

References Cited in the file of this patent

UNITED STATES PATENTS

|           |          |       |                |
|-----------|----------|-------|----------------|
| 2,451,420 | Watkins  | ----- | Oct. 12, 1948  |
| 2,517,694 | Merion   | ----- | Aug. 8, 1950   |
| 2,601,254 | Bruson   | ----- | Jan. 24, 1952  |
| 2,611,929 | Hoxie    | ----- | Sept. 20, 1952 |
| 2,715,763 | Marley   | ----- | Aug. 23, 1955  |
| 2,790,700 | Stanton  | ----- | Apr. 30, 1957  |
| 2,922,692 | Messer   | ----- | Jan. 26, 1960  |
| 2,948,581 | Cummings | ----- | Aug. 9, 1960   |